

United States Patent [19]  
Colwell

[11] 3,864,223  
[45] Feb. 4, 1975

[54] METHOD OF REGENERATION SPENT  
IRON ELECTROPLATING SOLUTIONS  
WITH CONCOMITANT DESULFURIZATION  
OF COAL

[75] Inventor: Robert E. Colwell, Palos Park, Ill.

[73] Assignee: Continental Can Company, Inc.,  
New York, N.Y.

[22] Filed: Mar. 21, 1973

[21] Appl. No.: 343,330

[52] U.S. Cl. 204/48, 44/1 R, 210/60,  
210/75, 423/153, 423/460, 423/461, 423/571

[51] Int. Cl. C101 9/02, C23b 5/04, C01b 17/02

[58] Field of Search 210/60, 75, 44/1 R;  
201/17; 423/153, 460, 461, 571; 204/48,  
237, 238, 239, 112, 113

[56] References Cited

UNITED STATES PATENTS

2,653,905 9/1953 Aannerud 204/112

2,726,148 12/1955 McKinley et al. 44/1 R  
3,768,988 10/1973 Meyers 44/1 R

OTHER PUBLICATIONS

R. E. Brewer et al., Ind. & Eng. Chem., Vol. 41, No.  
9, p. 2044, (1949).

Primary Examiner—G. L. Kaplan

Attorney, Agent, or Firm—Paul Shapiro; Joseph E.  
Kerwin; William A. Dittmann

[57] ABSTRACT

Spent iron electrolyte solutions withdrawn from iron plating baths containing  $Fe^{3+}$  are regenerated by centrifugally contacting the electrolyte with a bed of coal particles containing iron sulfides centrifugally fixed on the perforated sidewalls of a rotating reaction chamber. The process causes the rapid reduction of the  $FeCl_3$  to  $FeCl_2$  with the concomitant removal of the iron sulfides from the coal.

4 Claims, 1 Drawing Figure



PATENTED FEB 4 1975

3,864,223



**METHOD OF REGENERATION SPENT IRON  
ELECTROPLATING SOLUTIONS WITH  
CONCOMITANT DESULFURIZATION OF COAL**

**BACKGROUND OF THE INVENTION**

**1. Field of the Invention**

The present invention is directed to the regeneration of spent iron plating electrolyte solutions and more particularly to the regeneration of spent electrolyte solutions using coal particles having substantial iron pyrite content.

**2. The Prior Art**

Combustion of coal for heat, steam, and electrical power generation is by far the largest single source of atmospheric sulfur dioxide pollution in the United States; it currently accounts for about two thirds of the total sulfur oxide emissions. Federal government standards limit the discharge of sulfur dioxide into the atmosphere to 1.2 pounds per million Btu's of heat input for solid fossil fuel combustion operations generating more than 250 million Btu's per hour. This emission limit corresponds to a maximum sulfur content restriction of 0.6 - 0.8 percent for most Eastern coals. However, coal for utility consumption averages about 2.5 - 3.0 percent sulfur. The sulfur contained in the coal exists principally as ferrous sulfide ( $FeS_2$ ) commonly referred to as iron pyrites.

One method known to the art for the removal of iron pyrites is the Meyers process wherein the iron pyrites are leached from coal utilizing aqueous solutions of ferric ions, "Chemical Removal of Pyritic Sulfur from Coal" by J. M. Hamersa et al, Symposium on Environmental Pollution Control, American Chemical Society Division of Fuel Chemistry, Aug. 29-31, 1972, New York, N.Y.

In the Meyers process, coal containing iron pyrites is treated with an aqueous ferric chloride or sulfate solution at approximately 100°C to convert the pyritic sulfur content to elemental sulfur and  $Fe^{2+}$ . The aqueous solution is separated from the coal and the coal is washed to remove residual ferrous and ferric salt. The elemental sulfur which is dispersed in the coal matrix is then removed by vacuum distillation or extraction with a solvent such as toluene or kerosene. The resulting coal has a substantially reduced pyrite content and may be used as low sulfur fuel.

The chemical removal of iron pyrites using this process can be represented as follows:



It is also well known to the art as for example, U.S. Pat. Nos. 1,412,174, 1,862,745, 2,223,928, 2,316,917, 2,420,403 and U.S. Pat. No. 2,758,950, to electroplate iron articles such as sheets, foil, strips, tubes and the like wherein the iron is plated from an electroplating bath onto a suitably shaped cathode. Typically, the electroplating is accomplished with a highly concentrated  $FeCl_2$  solution. In the electroplating of iron using  $FeCl_2$  solutions, the cathode reaction is represented by the equation:



and the anode reaction by the equation:



The commercial applications of electroplating iron structures are readily apparent. The direct production of iron sheet, tubes or containers from iron plating baths would replace the capital and energy costs of the blast furnaces, rolling mills and shaping equipment presently required for the production of these iron articles. Utilizing scrap iron derived from discarded automobiles, metal containers and the like would permit recycling of these materials and thereby alleviate the serious ecological problem of solid waste disposal with which our nation is presently confronted.

Although it has been long known that iron can be deposited from its solutions by electrolysis and the commercial aspects of iron electroplating readily apparent, the process has been little used except in the building up of undersized parts and in the production of high purity iron.

One problem encountered in the electroplating of iron articles which has retarded the commercial application of the process is that the plating reaction rapidly depletes  $Fe^{2+}$  from the electrolyte and fresh electrolyte must be continuously fed to the electrolytic bath.

Methods of regenerating the spent electrolyte are complex and costly.

One method of regenerating spent electrolyte is disclosed and claimed in copending patent application Ser. No. 300,071 filed Oct. 24, 1972, the disclosure of which is incorporated in the present application by reference.

In the method disclosed in patent application Ser. No. 300,071, iron particles and spent  $FeCl_3$  electrolyte solution from an iron electroplating bath are charged to a rotating reaction chamber having sidewalls provided with a plurality of openings, the openings being of a size which is smaller than the size of the iron particles charged to the chamber. The chamber is rotated at a speed sufficient to cause the iron particles to be propelled outwardly under the influence of centrifugal force against the sidewalls of the chamber and to be fixed thereon to form a continuous bed of iron particles. The spent electrolyte solution charged to the chamber is propelled outward into contact with the iron particle bed and is caused to contact and move radially therethrough under the action of the same centrifugal force which fixes the particles on the chamber sidewalls. As the liquid reactant passes through the particle bed it reacts with the particle bed at an extremely high reaction rate in accordance with the equations:



The  $FeCl_2 + H_2$  reaction products then exit the chamber through the sidewall openings and are recovered.

**SUMMARY OF THE INVENTION**

In accordance with the present invention, there is provided a process for effecting the removal of iron sulfide from coal using spent electrolyte solution from iron plating baths wherein the spent electrolyte and coal particles containing iron sulfides are charged to a reaction chamber having a plurality of openings in its sidewalls, the size of the openings being smaller than the size of the coal particles. The chamber is rotated with sufficient rotational speed to generate a centrifugal force to cause the coal particles to be propelled out-

wardly against the walls of the chamber and be fixed thereon to form a continuous bed of particles. As the chamber is rotated, the spent electrolyte is propelled outward into contact with the coal particle bed fixed on the walls of the chamber and is caused to move radially therethrough under the action of centrifugal force, the spent iron electrolyte during its passage through the particle layer entering into chemical reaction with the iron sulfides contained in the coal particles whereby the iron sulfides are converted in to  $\text{FeCl}_2$  and sulfur. In the case of  $\text{FeS}_2$  the reaction proceeds in accordance with the equation:  $\text{FeS}_2 \cdot \text{Coal} + 2 \text{FeCl}_3 \rightarrow 3 \text{FeCl}_2 + 2 \text{S}$

The coal, after contact with the electrolyte is advanced through the reaction chamber by an oscillating pusher plate or other means, is washed to remove electrolyte, and is then discharged from the chamber.

#### DESCRIPTION OF THE DRAWING

The FIGURE is an elevational view, in vertical section, schematically showing the essential construction and arrangement of a centrifugal apparatus suitable for use in the practice of the present invention.

#### PREFERRED EMBODIMENTS

Referring now to the FIGURE, there is shown a centrifugal reactor 18 having a reaction chamber 19 operatively connected to a rotatable shaft 20 which is mounted in bearing 21 and is driven by a power source (not shown). A casing 23 encloses the reaction chamber 19. Inlet pipe 24 provides means whereby a slurry of coal particles 26 of a predetermined size and containing about 0.2 to 20 % or more iron pyrite mixed with spent electrolyte solution obtained from an iron plating bath are charged to the chamber 19.

The reaction chamber 19 is formed of a cylindrical perforated side wall 29 having a plurality of spaced openings 30 which are smaller in size than the size of the coal particles 26 fed to the chamber. Mounted within shaft 20 and adapted to oscillate within the chamber interior is distributor plate or disc 31. As the chamber 19 is caused to rotate about its axis by the rotation of the shaft 20, the coal particles supplied to the chamber interior 34 are caused to contact the rotating disc 31 and are continuously propelled radially outward toward and onto the perforated walls of the chamber by the centrifugal force exerted thereon. As the particles are of a size larger than the wall openings, the particles cannot penetrate the wall and remain fixed thereto as a continuous layer or bed of particles 32. Plate 31 is caused to oscillate periodically, pushing the bed of coal particles toward discharge means 25 of the chamber 19. The spent electrolyte entering the interior chamber 34 upon impingement on the rotating disc 31 is thrown radially outward against the particle bed 32 fixed to the wall 29 by the centrifugal force generated by the rotating chamber 19. When the chamber 19 is rotated at a speed which generates sufficient centrifugal force to keep the particles 26 in fixed alignment with the walls 29 of the chamber 19, the same centrifugal force causes the liquid electrolyte to move radially through the bed 32. As the electrolyte moves through the bed 32, the iron pyrite contained in the coal particles is converted to  $\text{FeCl}_2$  and S by reaction with the  $\text{FeCl}_3$  dissolved in the electrolyte.

The treated coal particles having the iron pyrites removed therefrom and discharged from the reactor

chamber are collected by suitable collection means, not shown. The sulfur is easily separated from the coal particles by washing or other conventional separation means.

5 The coal and electrolyte slurry feed rate and rotational speed of the chamber 19 are generally selected so that only a fraction of the interstitial pore volume of the bed is filled with liquid electrolyte at any given time, and flooding of the bed is thereby avoided.

10 At a constant slurry feed rate, the bed fillage can be readily reduced by increasing the chamber rotational speed.

15 After being propelled through the particle bed 32, the regenerated electrolyte, comprised of substantially reduced concentrations of  $\text{Fe}^{3+}$  and increased concentrations of  $\text{FeCl}_2$ , is continuously expelled by the action of the centrifugal force from the interior chamber 34 through the spaced openings 30 in the side wall 29 and enters the chamber 35. The regenerated electrolyte is caused to outwardly flow from the chamber 35 by gravity or by pumping and is discharged from the chamber 35 through outlet 36 provided in the bottom of the chamber 35.

20 25 The regenerated electrolyte discharged from the chamber 35 through the outlet 36, may be recycled through the same or a series of similar centrifugal reactors if more complete reduction of the  $\text{Fe}^{3+}$  ion is desired or the regenerated electrolyte may be immediately purified to remove contaminants and pumped directly into the electrolyte supply means of an electrolytic cell to provide fresh electrolyte for the iron plating reaction.

30 35 Alternative to the treatment of coal containing iron pyrites, the coal can be first mechanically cleaned and the coal refuse roasted converting its iron pyrite ( $\text{FeS}_2$ ) content to  $\text{FeS}$  in accordance with the equation:



40 45 The roasted coal refuse can then be contacted with  $\text{FeCl}_3$  solution in the centrifugal reactor 18 just described to effect the removal of the  $\text{FeS}$  content in accordance with the equation:  $\text{FeS} + 2 \text{FeCl}_3 \rightarrow 3 \text{FeCl}_2 + \text{S}$

50 55 What is claimed is:

1. A process for effecting the regeneration of spent electrolyte solutions obtained from iron plating baths comprising the steps of:

charging coal particles containing iron sulfides to a reaction chamber having a plurality of openings in its sidewalls, the size of the openings being smaller than the size of the particles,

rotating the chamber with sufficient rotational speed to generate a centrifugal force to cause the particles to be propelled outwardly against the walls of the chamber and be fixed thereon to form a continuous bed of particles,

charging spent electrolyte solution comprised of an aqueous solution of  $\text{Fe}^{3+}$  to the rotating chamber, the electrolyte solution being propelled outward into contact with the particle bed fixed on the walls of the chamber and caused to move radially therethrough under the action of centrifugal force, the  $\text{Fe}^{3+}$  in the electrolyte solution during the passage of the solution through the particle layer entering into chemical reaction with the iron sulfide contained in the particles whereby the  $\text{Fe}^{3+}$  of the elec-

trolyte and the iron sulfide is converted to  $Fe^{2+}$  and S.  
2. The process of claim 1 wherein the  $Fe^{3+}$  in the electrolyte solution is present as  $FeCl_3$  which is converted to  $FeCl_2$ .

3. The process of claim 1 wherein the coal contains  $FeS_2$ .  
4. The process of claim 1 wherein the coal contains FeS.

\* \* \* \* \*